

Patented Feb. 12, 1924.

1,483,087

# UNITED STATES PATENT OFFICE.

ROY LINDEN HILL, OF TAMAQUA, PENNSYLVANIA, ASSIGNOR TO ATLAS POWDER COMPANY, OF WILMINGTON, DELAWARE, A CORPORATION OF DELAWARE.

## AMMONIUM-NITRATE EXPLOSIVE.

No Drawing.

Application filed March 21, 1923. Serial No. 626,590.

To all whom it may concern:

Be it known that ROY LINDEN HILL, citizen of the United States, residing at Tamaqua, in the county of Schuylkill and State of Pennsylvania, has invented certain new and useful Improvements in Ammonium-Nitrate Explosives, of which the following is a specification.

My invention relates to ammonium nitrate explosives of varying strengths and properties, particularly adapted for use in commercial blasting work, but well suited for use in other relations.

For many years ammonium nitrate has been a constituent of varied types of commercial and military explosives. It has been substituted for part of the nitroglycerine of so-called straight dynamites and ammonia gelatin dynamites of commerce. The prime object of this substitution has been cost reduction, other accomplishments being somewhat greater safety in handling and somewhat less ease of ignition. However, they contain eight per cent or more of nitroglycerine or equivalent in order that their properties may not differ too greatly from the equivalent straight grades. They may, therefore, cause severe headaches to those handling them in the course of manufacture and use. They may also become hard, insensitive and dangerous to handle through crystallization of the nitroglycerine under the influence of cold, the so-called frozen dynamite effect. Various more or less efficient

means have been used to increase their freezing resistance, such as the use of nitrated carbohydrates, tetranitrodiglycerine and nitro-aromatic compounds in conjunction with nitroglycerine, but they will all become hard due to a crystallization of nitroglycerine under certain existing climatic conditions. Further, ammonium nitrate is a prime ingredient in many of the permissible (for use in coal mines) explosives. In one type it is used in connection with five per cent or more nitroglycerine together with relatively small amounts, on occasion, of such materials as sodium chloride, ammonium chloride, sodium nitrate, wood pulp, materials added to depress the freezing point of nitroglycerine, etc. These explosives possess the disadvantages enumerated under ammonia dynamites. In another type, which is not necessarily confined to permissible explosives, it is used in connection with

sensitizers, such as non-explosive carbonaceous matter, nitro-aromatic compounds, or powdered metals, usually with the addition of some material to reduce the temperature of detonation or length of flame, if the explosive is to be permissible. This type has been very unsatisfactory in application because of insensitiveness and frequent failure to detonate or at least propagate detonation. Sensitiveness might be increased through the introduction of large amounts of nitro-aromatic compounds, but the result is excessive cost and quantities of poisonous gases in the products of detonation. A modification of this type to improve sensitiveness and eliminate excessive amounts of poisonous gases in the products of detonation has consisted in using a small amount of nitro-aromatic compounds, 17% or less, and introducing a small percentage of nitroglycerine as sensitizer. Thus there is a very limited sensitizing effect due to the nitro-aromatic and considerable amounts of nitroglycerine must be used to insure a satisfactory condition of sensitiveness, with resultant disadvantages on this account.

Ammonium nitrate is also used in conjunction with nitro-starch as a commercial and military explosive and in conjunction with T. N. T. as a shell bursting charge for military purposes. Many other combinations might be proposed or may have been used to a limited extent for special purposes.

By extensive thought and experimentation I have been able to devise a series of ammonium nitrate explosives which nearly or entirely eliminate the objections to previous types. I obtain economy in manufacture and ingredients, a satisfactory degree of propagation sensitiveness, a wide range in strength, a good condition as regards poisonous gases on detonation in the accepted sense, freedom from headaches in handling, except slight, hardly noticeable ones to a few most susceptible persons, and freedom from becoming hard and insensitive through crystallization of nitro-glycerine under any climatic conditions met in practice. I have developed by actual test with many persons that, in the case of explosives of nitroglycerine content below ten per cent, susceptibility to nitroglycerine headaches and the severity of the same decline proportionately with decrease in nitroglycerine

content, that three and one-half per cent inconveniences one of these persons and that four and one-half per cent was the maximum at which most persons would feel no inconvenience. I have further been unable under any conditions of cold met in practice to cause my explosives to become hard through crystallization of nitroglycerine, except in the case of a special adaptation 10 for warm weather use, to be noted later.

My explosives are made on the basis that strength is varied essentially by varying the amount of ammonium nitrate, that nitro-aromatics of which at least 50% is trinitrotoluene are used in an amount sufficient to contribute appreciable sensitiveness yet not in amount sufficient to prevent a satisfactory condition as regards poisonous gases on detonation, that one and one-half to 20 four and one-half per cent liquid organic nitrate is used to reduce the dustiness and as a contributory sensitizer and that a non-explosive inorganic nitrate is used as a filler and to provide oxygen as desired.

Other well known ingredients of a non-explosive, but combustible nature may be used on occasion. Examples might be mentioned as sulphur, flour and ground wood. Summarizing, my explosives consist of 30 seventeen to thirty-two per cent (17-32%) nitro-aromatics of which at least 50% is trinitrotoluene, one and one-half to four and one-half per cent (1½-4½) liquid organic nitrate or liquid mixtures of organic nitrates, ammonium nitrate in sufficient quantity to give the desired strength and non-explosive inorganic nitrates in sufficient quantity to act as filler or to furnish the desired amount of oxygen. Incidental 40 ingredients of an inert or non-explosive combustible nature may be added as antacid, filler or to assist in balancing such properties as oxygen content, and density, but these do not essentially alter the properties of my explosives.

It is especially to be understood that "liquid organic nitrate" as used in the claims is broad enough to cover a single nitrate or a mixture of nitrates.

Typical formulae, by way of example, are:

|                                                        |      |      |      |
|--------------------------------------------------------|------|------|------|
| Ammonium nitrate-----                                  | 52.5 | 32.5 | 17.5 |
| Mixture of nitroglycerine<br>and tetranitrodiglycerine | 3    | 3    | 3.5  |
| Sodium nitrate-----                                    | 24   | 40   | 52.5 |
| Chalk -----                                            | 0.5  | 0.5  | 0.5  |
| Nitro-aromatics -----                                  | 20   | 24   | 24   |
| Sulphur -----                                          | 2    |      |      |

The fact that both ammonium nitrate and nitro-aromatics are explosive ingredients and consequently exert a sensitizing effect makes it possible to use a very limited amount of liquid organic nitrate sensitizer and yet obtain a practical degree of sensitiveness. The fact that I do use a small

amount of liquid organic nitrate renders it unnecessary to use excessive amounts of the uneconomical (strength for cost) and highly oxygen deficient nitro-aromatics. Ammonium nitrate, which is an economical 70 strength producer and contains an excess of oxygen, fits into this combination as a simple, convenient and economical means of producing a wide variety of explosive strengths. Sodium nitrate is a relatively 75 cheap filler and producer of oxygen on detonation of the explosives.

While, as liquid organic nitrate, I have shown in the examples a mixture of nitroglycerine and tetranitrodiglycerine, I may 80 also use nitroglycerine (glycerin trinitrate) only where resistance to cold is not an object, or where cold resistance is desired, I may use mixtures of glycerin trinitrate with other organic nitrates which depress its solidifying point and which forms a liquid mixture with it, such as the glycol dinitrates, chlorhydrin dinitrates, and nitrated carbohydrates, or I may use liquid organic nitrates, exclusive of glycerin trinitrate.

I am aware of the extended use of ammonium nitrate in explosives, but in so far as I can ascertain by consultation of patents and of the literature and by examination of 95 many explosives compositions which are being produced, I believe that I am the first to prepare the peculiar combination of ingredients herein set forth which so largely offsets many of the disadvantages of previous types of ammonium nitrate explosives. My investigations indicate that I have combined the good points of several previous types with the elimination of most of the 100 bad points, the result being a new general 105 type of great flexibility and practical advantage.

Having described my invention what I claim is:

1. An ammonium nitrate explosive containing 17 to 32% nitroaromatics of which at least 50% is trinitrotoluene, a non-explosive inorganic nitrate and a liquid organic nitrate.
2. An ammonium nitrate explosive containing 17 to 32% of nitroaromatics of which at least 50% is trinitrotoluene, sodium nitrate and a liquid organic nitrate.
3. An ammonium nitrate explosive containing 17 to 32% nitroaromatics of which at least 50% is trinitrotoluene, a non-explosive inorganic nitrate and 1½ to 4½% of liquid organic nitrate.
4. An ammonium nitrate explosive containing 17 to 32% nitroaromatics of which at least 50% is trinitrotoluene, sodium nitrate and 13 to 4½% of liquid organic nitrate.
5. An ammonium nitrate explosive containing 17 to 32% nitroaromatics of which 130

at least 50% is trinitrotoluene, sodium nitrate and 1 $\frac{1}{2}$  to 4 $\frac{1}{2}$ % of a mixture of glycerine trinitrate and diglycerine tetrinitrate.

6. Ammonium nitrate explosives containing 17 to 32% nitroaromatics of which at least 50% is trinitrotoluene and 1 $\frac{1}{2}$  to 4 $\frac{1}{2}$ % of liquid organic nitrate, with ammonium nitrate and non-explosive inorganic nitrates in such proportions that various strengths and desired oxygen conditions are obtained.

7. Ammonium nitrate explosives containing 17 to 32% nitroaromatics of which at least 50% is trinitrotoluene and 1 $\frac{1}{2}$  to 4 $\frac{1}{2}$ % of liquid organic nitrate, with ammonium nitrate and sodium nitrate.

8. Ammonium nitrate explosives contain-

ing 17 to 32% nitroaromatics of which at least 50% is trinitrotoluene, 1 $\frac{1}{2}$  to 4 $\frac{1}{2}$ % of liquid mixture of organic nitrates, sodium nitrate, and non-explosive combustible material.

9. Ammonium nitrate explosives containing 17 to 32% trinitrotoluene, 1 $\frac{1}{2}$  to 4 $\frac{1}{2}$ % of liquid organic nitrate, sodium nitrate and non-explosive combustible material. 25

In testimony whereof he affixes his signature in the presence of two witnesses.

ROY LINDEN HILL.

Witnesses:

MABEL R. HILL,  
RUSSELL M. COOK.